

Patented Aug. 15, 1939

2,169,690

# UNITED STATES PATENT OFFICE

2,169,690

## FIBER

Stephen P. Gould and Earle O. Whittier, Washington, D. C.; dedicated to the free use of the People in the territory of the United States

No Drawing. Application May 28, 1938,  
Serial No. 210,789

2 Claims. (Cl. 18—54)

(Granted under the act of March 3, 1883, as  
amended April 30, 1928; 370 O. G. 757)

This application is made under act of March 3, 1883, as amended by the act of April 30, 1928, and the invention herein described and claimed, if patented, may be manufactured and used by or for the Government of the United States of America for governmental purposes without the payment to us of any royalty thereon.

We hereby dedicate the invention herein described to the free use of the people in the territory of the United States to take effect on the granting of a patent to us.

Our invention deals with a precipitating bath useful for precipitating, strengthening, and rendering water-resistant, fibers composed essentially of casein.

The object of our invention is to produce a bath containing a soluble calcium (or other alkaline earth) compound which will react with the fibers to increase their strength and water-resistance, and to minimize loss of calcium from the fibers while they are in the precipitating bath.

Sulfuric acid is commonly used in said baths, but calcium cannot be incorporated with it because of the formation of insoluble calcium sulfate. Hydrochloric acid seems to exert a weakening effect on the fibers. However, we found that a combination of phosphoric acid and monocalcium phosphate  $[\text{CaH}_4(\text{PO}_4)_2 \cdot \text{H}_2\text{O}]$  worked well since the calcium was kept in soluble form in the bath.

The following example illustrates a satisfactory procedure. Proportions are given in parts.

### EXAMPLE 1

#### Spinning solution

|                       |       |
|-----------------------|-------|
| Casein                | 24    |
| Water                 | 208.8 |
| Sodium lauryl sulfate | 4.8   |
| Calcium hydroxide     | 2.4   |
| Water                 | 60    |

The 24 parts of casein are soaked in the 208.8 pts. of water for 15-30 minutes and the sodium lauryl sulfate is then stirred into the mixture.

In the meantime, a mixture of the 2.4 pts. of

calcium hydroxide and the 60 pts. of water should be prepared. This is next stirred mechanically into the casein mixture until a smooth dispersion is obtained. This solution requires careful filtration.

#### Precipitating bath

|                                                                                |    |
|--------------------------------------------------------------------------------|----|
| Phosphoric acid                                                                | 5  |
| Monocalcium phosphate $[\text{CaH}_4(\text{PO}_4)_2 \cdot \text{H}_2\text{O}]$ | 10 |
| Formaldehyde                                                                   | 5  |
| Dextrose                                                                       | 20 |
| Water                                                                          | 60 |

Spinning solution and bath temperatures were both 50° C., but temperatures varying from room to 80° C. may be employed.

The fibers thus produced showed unusually good strength, elasticity, and water-resistance. They may be improved by after-treating with oils.

It will be understood that our invention is not limited to this example as proportions, substitutes (such as barium hydroxide), and constituents may be varied over a wide range.

In making use of our precipitating bath, the general spinning procedures of the rayon industry are, of course, applicable. That is, the spinning solution is extruded into the precipitating bath, through any type of spinnerette normally used in the rayon industry.

Having thus described our invention what we claim for Letters Patent is:

We claim:

1. A process for producing casein fibers of enhanced strength and water resistance, which includes subjecting an alkaline solution comprising casein, in the form of fine streams, to the action of an acid bath comprising a solution of phosphoric acid and an alkaline earth phosphate.

2. A process for producing casein fibers of enhanced strength and water resistance, which includes subjecting an alkaline solution comprising casein, in the form of fine streams, to the action of an acid bath comprising a solution of phosphoric acid and monocalcium phosphate.

STEPHEN P. GOULD.

EARLE O. WHITTIER.